

## UNITED STATES PATENT OFFICE

2,058,342

PETROLEUM LUBRICANT PRODUCT AND  
METHOD OF MAKING SAME

Robert C. Moran, Wenonah, and William L. Evers and Everett W. Fuller, Woodbury, N. J., assignors to Socony-Vacuum Oil Company, Incorporated, New York, N. Y., a corporation of New York

No Drawing. Application October 3, 1935,  
Serial No. 43,328

4 Claims. (Cl. 87—9)

Recent changes in automotive engine design, tending toward higher bearing pressures, higher rotative speeds, higher engine temperatures, and the like, have occasioned departure from the use 5 of the usual bearing metals such as babbitt. The newer bearing metals are of different nature and, while harder, are in general more susceptible to 10 destructive agencies of a corrosive nature. Typical of these newer bearings are those composed of a cadmium-silver alloy supported upon a steel back, which are now widely installed in certain 15 makes of automobiles. Others of these relatively new bearing metals which may be mentioned are cadmium-nickel and copper-lead alloys.

15 These changes in engine design have been concurrent with marked advances in methods of refining lubricant oils for automotive use. The demand for oils having lesser changes in viscosity 20 with temperature change; i. e., higher viscosity index (V. I.) has been met by refining lubricants intended for motor oils by certain solvent refining or solvent extraction processes, wherein advantage is taken of the selective solvent power for 25 hydrocarbons of various types which is possessed by certain liquid reagents, for example, dichloro-diethylether, cresylic acid, phenol, chloraniline, chlorophenol, phenetidine, benzyl alcohol, nitrobenzene benzonitrile, furfural, aniline, benzyl acetate, liquid sulfur dioxide, mixtures of liquid sulfur dioxide or aniline with benzol, and the like. 30 These solvent refining processes are operated to concentrate in the desired lubricant fraction those compounds of a "paraffinic" nature possessed of the ability to suffer only a small change 35 of viscosity upon change of temperature, and to reject the compounds of "naphthenic" nature which do suffer such change of viscosity to a more marked degree. These refining processes have enabled supply of an oil of quite desirable general 40 characteristics, definitely far superior to any oil previously produced from mixed base or asphaltic crudes, and superior to a like, though lesser, degree over oils previously produced from paraffine base crudes.

45 It has been found that the solvent refined motor oils referred to above are for some reason definitely corrosive to the newer bearing metals under normal conditions of automotive use, sometimes resulting in bearing failure after only a few thousand miles of normal driving. It is further known that the same reaction, viz, corrosion of 50 alloy bearing metals such as cadmium-silver, also occurs in good paraffinic base oils which have not been subjected to solvent refining. The higher 55 the V. I. of the lubricating oil, the more pronounced

is the tendency to corrosion of the kind referred to above. Generally speaking, the problem is encountered in oils having a V. I. of 75 or higher, and becomes important in oils having a V. I. of 80 to 85 or higher, and very important in oils of 100 V. I. or 5 higher.

It is an important object of this invention to provide means for satisfactorily inhibiting or preventing this corrosion from taking place to a serious degree. It is an object of this invention to alter or modify a highly refined motor oil, normally corrosive, by the use of an additive ingredient capable of substantially inhibiting this corrosion. It is an object to provide a substantially 10 non-corrosive motor oil of high V. I. An object of this invention is to provide an additive reagent or ingredient capable of inhibiting the corrosive properties of these oils. The production of solvent refined oils of low corrosive properties under 15 conditions of automotive use is a major object of this invention, as well as the method of production of such oils which couple high viscosity index 20 with low tendency to corrosion.

25 This invention is based upon the discovery that addition to the oil of small amounts of triphenylphosphite ( $C_6H_5O$ )<sub>3</sub>P accomplishes the above objects. It is found that when corrosion of the type outlined above occurs, especially if the oil be one which has been produced by a process of solvent refining, in which type the corrosive properties 30 appear to be the most marked, that the oil can be rendered substantially non-corrosive under conditions more strenuous than normal automotive use by the addition of controlled amounts of 35 this compound, viz, triphenylphosphite.

35 Triphenylphosphite is an organic compound having the following graphic formula:



40 This compound may be prepared by the reaction of phenol and phosphorus trichloride, in the proportions of three molecular amounts of phenol to one of phosphorus trichloride. The reaction mixture is heated until the evolution of hydrogen chloride ceases. This evolution of HCl gas 45 may be measured, since it furnishes a convenient means of estimating and controlling the progress of the reaction. The resulting product, triphenylphosphite, may be purified, if desired, by 50 a process of fractional distillation, the pure com- 55

- 5 pound boiling at 209-210° C. at 1 mm. mercury pressure. For the present objects it may be used either as produced or in the fractionated form, although the use of the fractionated compound  
 10 is preferred. A satisfactory reaction product may be made by heating the reaction mixture, after the cessation of the evolution of HCl gas, to a temperature of 190° C. under a pressure of 1 mm. mercury (designated herein as "Topped").  
 15 By fractionation, this may be conveniently made to yield a product boiling at 205-215° C. at 1 mm. mercury pressure (designated herein as "Fractionated").

15 The following sets of data demonstrate the effectiveness of this novel corrosion inhibitor. In all of these tests, the oil used was a solvent refined motor oil of SAE 20 rating, having a Saybolt viscosity of 56 seconds at 210° F., a flash point of 420° F., and a V. I. of 117. Actual motor 20 operation tests are set forth in Table I, below, four comparative tests being given. In these tests, a motor oil blank and motor oil blends containing different proportions of the novel inhibiting ingredient of this invention were subjected to test in a modified Delco knock test engine, equipped with bearings of cadmium-silver alloy on a steel back. The alloy is about 2.5% silver, a few hundredths of a per cent of copper, and the 25 balance of cadmium. The motor was equipped with crankcase oil heaters to maintain oil-temperatures (330° F.) at least equal to those encountered under extreme conditions of automotive use. On each test the test engine was operated for 20 hours at a rotative speed the equivalent of an automobile road speed of 60 miles per hour. In rough terms, each test is the equivalent of exposure of the oil to use in an automobile for 1200 miles of continuous 60 mile an hour driving, a condition far more rigorous than any 30 encountered in normal use. The bearings in the engine were new for each test, and were carefully weighed before and after to determine loss in weight. The neutralization number (N. N.) of 35 the used oil was measured, and is recorded as being indicative of the corrosive nature of the oil. The inhibitor used was the fractionated triphenylphosphite of 205-215° C. boiling point at 40 1 mm. mercury pressure described above.

50 TABLE I  
 Engine tests

| 55                          | Test | Bearing loss, milligrams | N. N. of used oil |
|-----------------------------|------|--------------------------|-------------------|
| Oil alone.....              | 5916 | 4.9                      |                   |
| Oil + 0.50% ingredient..... | 48   | 0.1                      |                   |
| Oil + 0.25% ingredient..... | 55   | 0.1                      |                   |
| Oil + 0.10% ingredient..... | 3207 | 3.0                      |                   |

60 From this it may be seen that the use of this novel corrosion inhibitor, viz, triphenylphosphite, in amounts as small as one quarter of one per cent prevented corrosion to a substantially complete degree under conditions much more rigorous than any likely to be met in practice, while as little as one tenth of one percent reduced the bearing loss almost one half.

65 An indicative test of considerable merit may be made in the laboratory by suspending a portion of a cadmium-silver alloy bearing in a bath of the oil under test in a glass container, maintaining the oil at about 350° F., and passing air through the oil in contact with the bearing metal. Convenient 70 conditions are: 30 gm. oil, 2,000 ml. air per hour, 22

hours. The following table shows results of a series of such tests in which oils containing different proportions of triphenylphosphite, and an oil blank were tested, giving the loss in weight of the bearing metal, and the neutralization number of the used oil. The oil used was the same as in Table I.

10 TABLE II  
 Corrosion tests in glass

| Test                                       | Bearing loss, milligrams | N. N. of used oil | 15 |
|--------------------------------------------|--------------------------|-------------------|----|
| Oil Alone.....                             | 30                       | 1.8               |    |
| Oil + 2.00% ingredient (Fractionated)..... | 1                        | 0.5               |    |
| Oil + 1.00% ingredient (Fractionated)..... | 0                        | 0.5               |    |
| Oil + .50% ingredient (Fractionated).....  | 0                        | 0.8               |    |
| Oil + .25% ingredient (Fractionated).....  | 1                        | 0.8               |    |
| Oil + .10% ingredient (Fractionated).....  | 1                        | 0.5               |    |
| Oil + .05% ingredient (Fractionated).....  | 8                        | 1.0               | 20 |
| Oil + .10% ingredient (Topped).....        | 0                        | 0.5               |    |
| Oil + .05% ingredient (Topped).....        | 13                       | 1.2               |    |

25 From the combined evidence of the above exemplary data, it is evident that the novel corrosion inhibiting ingredient herein disclosed, namely triphenylphosphite, is an effective agent for the prevention of corrosion of automotive parts, particularly the newer type alloy bearings, when introduced in proper amounts into an oil otherwise highly corrosive.

30 Visual examination of the bearings from engine tests such as those reported in Table I show the effectiveness of triphenylphosphite in a very marked manner. The bearing subjected to the oil blank shows plainly the effect of corrosion, very little of the original surface remaining. The bearings subjected to the inhibited oils show little or no visual evidence of corrosion. Similar visual 35 evidence of the effectiveness of this inhibitor may be noted by inspection of the pieces of metal used in the tests in glass.

40 It is preferred to use this ingredient, triphenylphosphite, in amounts ranging between 0.25% and 1.0% although for less severe services and in oils not highly corrosive, as low as 0.10% may be fully effective for the purposes intended.

45 This ingredient, triphenylphosphite, is a water clear oil, freely miscible with hydrocarbons, and may be added in any proportion without darkening or deepening the color of the oil. When so added, it has no tendency to separate from the oil under conditions of storage or use.

50 We claim:

55 1. A method of lubricating bearing surfaces in internal combustion engines when subjected to conditions of operation which comprises maintaining between bearing surfaces, one of which is an alloy formed chiefly of a metal selected from the class consisting of cadmium and copper, a film of lubricating oil which initially produces an effective lubricating action but which would normally tend to corrode the aforesaid alloy, and maintaining the effectiveness of the lubricating oil by incorporating therein triphenylphosphite in a small but sufficient proportion substantially to retard the corrosion.

60 2. A method of lubricating bearing surfaces in internal combustion engines when subjected to conditions of operation which comprises maintaining between bearing surfaces, one of which is an alloy formed chiefly of a metal selected from the class consisting of cadmium and copper, a film of lubricating oil which initially produces an effective lubricating action but which would normally tend to corrode the aforesaid alloy, and

70

75

80

85

90

95

100

105

maintaining the effectiveness of the lubricating oil by incorporating therein from 0.1% to 1.0% of triphenylphosphite sufficient substantially to retard the corrosion.

- 5 3. A method of lubricating bearing surfaces which comprises maintaining between bearing surfaces, one of which is an alloy selected from the class consisting of cadmium-silver, cadmium-nickel, and copper-lead alloys a film of lubricating oil which initially produces an effective lubricating action but which would normally tend to corrode the aforesaid alloy, and maintaining the effectiveness of the lubricating oil by incorporating therein triphenylphosphite in a small but 10 sufficient proportion substantially to retard the corrosion.
- 10 4. A method of lubricating bearing surfaces which comprises maintaining between the bearing surfaces, one of which contains a characterizing proportion of cadmium, silver, nickel, copper or lead, a film of lubricating oil which initially produces an effective lubricating action but which would normally tend to corrode the aforesaid surface, and maintaining the effectiveness of the lubricating oil by incorporating therein triphenylphosphite in a small but sufficient proportion to 15 substantially retard the corrosion.

ROBERT C. MORAN.  
WILLIAM L. EVERE.  
EVERETT W. FULLER. 15

### Certificate of Correction

Patent No. 2,058,342.

October 20, 1936.

ROBERT C. MORAN ET AL.

It is hereby certified that error appears in the printed specification of the above numbered patent requiring correction as follows: Page 1, second column, lines 38 to 44, inclusive, strike out the formula and insert instead the following:



and that the said Letters Patent should be read with this correction therein that the same may conform to the record of the case in the Patent Office.

Signed and sealed this 23rd day of February, A. D. 1937.

[SEAL]

HENRY VAN ARSDALE,  
*Acting Commissioner of Patents.*

**Certificate of Correction**

Patent No. 2,058,342.

October 20, 1936.

ROBERT C. MORAN ET AL.

It is hereby certified that error appears in the printed specification of the above numbered patent requiring correction as follows: Page 1, second column, lines 38 to 44, inclusive, strike out the formula and insert instead the following:



and that the said Letters Patent should be read with this correction therein that the same may conform to the record of the case in the Patent Office.

Signed and sealed this 23rd day of February, A. D. 1937.

[SEAL]

**HENRY VAN ARSDALE,**  
*Acting Commissioner of Patents.*